

Nov. 3, 1931.

H. T. REEVE

1,829,810

ELECTRON EMITTER

Filed Aug. 26, 1924

Fig. 1



Fig. 2



Fig. 3



Fig. 4



Fig. 5



Fig. 6



Inventor:  
Howard T. Reeve,  
by *Edward A. Adams, Atty*

## UNITED STATES PATENT OFFICE

HOWARD T. REEVE, OF MILLBURN, NEW JERSEY, ASSIGNOR TO WESTERN ELECTRIC COMPANY, INCORPORATED, OF NEW YORK, N. Y., A CORPORATION OF NEW YORK

## ELECTRON Emitter

Application filed August 26, 1924. Serial No. 734,218.

This invention relates to electron discharge devices and has for an object a thermionically active alloy and the process of making the same.

Many metals having high thermionic activity cannot be made into filaments because of their physical properties, while other metals possessing the requisite physical properties are not thermionically active.

Many metals having high thermionic activity cannot be made into filaments because of their physical properties, while other metals possessing the requisite physical properties are not thermionically active.

10 This invention contemplates combining metals of high melting point with metals having high thermionic activity to form alloys suitable for use as filaments in electron discharge devices.

15 Referring now to the drawings, the various figures thereof are illustrative of the steps in the process of forming a thermionically active filament according to this invention.

Fig. 1 is a sectional view of a suitable die and block for compressing the powdered material.

Fig. 2 is a section on line 2—2 of Fig. 1.

Fig. 3 is a section of a suitable furnace for subjecting the rod to heat treatment.

20 Fig. 4 is a side view of the swaging machine for hammering the rod into the form of wire.

25 Fig. 5 is a perspective view of the hammer used in the swaging machine, and

30 Fig. 6 is a sectional view of a die for drawing down the wire into the filamentary form.

The first step in the process comprises mixing together in powdered form, the oxide of a thermionically active metal and a reducing agent together with the high melting point metal to be alloyed. This mixture is compressed by means of the die 11 and block 12 shown in Figures 1 and 2 to form a rod 13. The rod is then subjected to heat treatment

35 in a vacuum or a hydrogen atmosphere in a furnace 14, such as disclosed in Figure 3.

This treatment reduces the thermionically active metal from its oxide while the reducing agent takes up the oxygen released from the oxide and is slagged off leaving an alloy of the high melting metal and thermionically active metal.

40 The process of making a thermionically active cathode for electron discharge devices which comprises combining a metal having a high melting point with alkaline earth oxides and a reducing agent, heating the same to reduce the alkaline earth oxide and oxidize the reducing agent, and working the resultant product into filamentary form.

45 The process of making a thermionically active cathode for electron discharge devices which comprises mixing alkaline earth oxides, aluminum and nickel, pressing said mixture into the form of a rod, heating said mixture in a vacuum to reduce the oxides and oxidize the reducing agent, separating aluminum oxide from the remainder and working the remainder into filamentary form.

In witness whereof I hereunto subscribe my name this 22d day of August, A. D. 1924.

HOWARD T. REEVE.

As a specific example, oxides of thermionically active metals such as barium and strontium may be mixed with aluminum as the re-



55

The reaction would be similar in case oxides of other alkaline earths or rare earths were used instead of barium oxide. Heat applied during the reaction fuses together the nickel and thermionically active metal to form an alloy. It is of course understood that the alloys formed may be composed of a metal of high melting point and one or more thermionically active metals.

60

The rods of nickel and strontium or barium are then hammered into the form of wire by means of the swaging machine 15 shown in Fig. 4, a hammer 16 of which is shown in Fig. 5. After being swaged into the form of wire, the alloy is drawn down into filamentary form by being passed through a succession of dies 17, such as shown in Fig. 6.

65

## What is claimed is:

1. The process of making a thermionically active cathode for electron discharge devices which comprises combining a metal having a high melting point with alkaline earth oxides and a reducing agent, heating the same to reduce the alkaline earth oxide and oxidize the reducing agent, and working the resultant product into filamentary form.

2. The process of making a thermionically active cathode for electron discharge devices which comprises mixing alkaline earth oxides, aluminum and nickel, pressing said mixture into the form of a rod, heating said mixture in a vacuum to reduce the oxides and oxidize the reducing agent, separating aluminum oxide from the remainder and working the remainder into filamentary form.

75

80

85

90

95

95

100